

# UNITED STATES PATENT OFFICE.

NATHAN DRESSER, OF ROCHESTER, NEW YORK.

## IMPROVEMENT IN LUBRICATING COMPOUNDS.

Specification forming part of Letters Patent No. 12,716, dated April 17, 1855.

*To all whom it may concern:*

Be it known that I, NATHAN DRESSER, of the city of Rochester, in the county of Monroe and State of New York, have invented a new and useful lubricating compound to prevent friction on car-journals, steamboat-cranks, carriage-axles, and all kinds of machinery subject to friction; and I do hereby declare that the following is a full and exact description thereof, reference being had to the accompanying lubricating compound.

The nature of my invention consists in making a lubricating compound which will run journals, cranks, axles, and other machinery in brass, composition, cast-iron, or wood boxes, or otherwise with a great saving of oil, grease, or other material now in use.

To enable others to make and use my invention, I will proceed to describe its compound and uses.

I make my lubricating compound by melting one pound of tallow, and while hot add half a pound of sperm or other oil. Then add two pounds of pure pulverized or granulated lead, with which, in warm weather, I use more tallow, and in cold weather more oil, to make

it of a sufficient consistence to hold the lead in suspension when applied to the boxes, journals, or other parts of machinery.

The lead is prepared in the following manner: I melt the pig or bar lead, and pour it off until I get the dross and other impurities from it. Then I melt it in an iron vessel, and as it cools I keep the lead at the sides thrown toward the center, so that it may cool equally, and with an iron stirring-rod I keep it briskly agitated until it granulates. Then, when cool, I sift out the fine particles, and so continue to melt and agitate until the whole is reduced to the aforesaid pulverized or granulated lead.

What I claim as my invention, and desire to secure by Letters Patent, is—

The lubricating compound and its application to journals, cranks, axles, and other machinery subject to friction, using for that purpose the aforesaid compound, or any other substantially the same, and which will produce the intended effect.

NATHAN DRESSER.

Witnesses:

W. C. CHACE,  
BARNEY BECKER.